

## UNITED STATES PATENT OFFICE

2,500,498

## LUBRICANT

Orland M. Reiff and Harry J. Andress, Jr., Woodbury, N. J., assignors to Socony-Vacuum Oil Company, Incorporated, a corporation of New York

No Drawing. Application July 11, 1946,  
Serial No. 682,929

2 Claims. (Cl. 252—46.6)

1

This invention has to do with the art of lubrication and, more particularly, has to do with lubricant compositions.

It is well recognized by those familiar with the art that lubricant compositions, such as viscous mineral oil fractions, tends to deteriorate when used in present day internal combustion engines. In such use, lubricant compositions develop substantial quantities of carbonaceous deposits which accumulate as sludge or "carbon deposits," thereby impairing the free flow of the oil. These deposits accumulate about the piston rings, causing them to stick. There is also developed in the oil, as the result of oxidation, appreciable acidity which has a deleterious effect upon metal parts with which the oil comes in contact. This is particularly severe in the case of certain types of alloy-bearing metals, such as copper-lead, cadmium-nickel, cadmium-silver, and the like. Additionally, the lubricating effectiveness of such lubricant compositions may be seriously reduced by virtue of the relatively large change in viscosity at engine operating temperatures.

We have now discovered that the foregoing shortcomings of lubricant compositions may be overcome substantially by the incorporation therein of small amounts of two characterizing agents which cooperate to provide a synergistic effect, rather than a mere additive effect. The characterizing agents which have this surprising cooperative action are oil-soluble phosphorus-containing compounds and oil-soluble compounds characterized by a thiophene nucleus.

The oil-soluble, phosphorus-containing compounds contemplated herein include the phosphites, phosphates, thiophosphites, thiophosphates, and their corresponding metal, ammonium and amine salts; phosphines; reaction products of phosphorus-containing reagents, such as phosphorus oxides, sulfides, halides, oxy- and thio-halides with various organic materials such as olefins, terpenes, alcohols, esters, ketones, acids, amines, etc.; phosphatides such as lecithin, cephalin, etc.; organo heterocyclic compounds containing phosphorus in the heterocyclic ring.

The typical phosphorus-containing characterizing agents are:

- (1) Phosphites
  - Amyl phenyl phosphite
  - Dibutyl phenyl phosphite
  - Triwax phenyl phosphite
- (2) Phosphates
  - Tricresyl phosphate
  - Lauryl phenyl phosphate
  - Triwax phenyl phosphate
- (3) Thiophosphites
  - Dibutyl thiophosphite
  - Tri xylene thiophosphite
  - Triwax phenyl thiophosphite
- (4) Thiophosphates
  - Tricresyl thiophosphate
  - Tri xylene thiophosphate
  - Triwax phenyl thiophosphate

2

- (5) Phosphines
  - Dibutyl phenyl phosphine
  - Dilauryl phenyl phosphine
  - Diwax phenyl phosphine
- (6) Phosphorus-containing reaction products of:
  - (a) Phosphorus oxides
    - $P_2O_3$ ,  $P_2O_5$
  - (b) Phosphorus sulfides
    - $P_2S_3$ ,  $P_2S_5$ ,  $P_4S_3$ ,  $P_4S_7$
  - (c) Phosphorus halides
    - $PCl_3$ ,  $PCl_5$ ,  $PBr_3$ ,  $POCl_3$ ,  $PSCl_3$
  - (d) Olefins
    - butylene, amylene, paraffin wax olefin
  - (e) Terpenes
    - pinene, camphene, turpentine oil
  - (f) Alcohols
    - octyl, decyl, lauryl, cetyl
  - (g) Ketones
    - phorone, dioleyl ketone
  - (h) Acids
    - stearic, oleic, salicylic
  - (i) Amines
    - amyl, stearyl, aniline
- (7) Phosphorus-containing natural products
  - lecithin, cephalin

The characterizing agent which cooperates with the aforesaid oil-soluble phosphorus-containing compounds is an oil-soluble compound characterized by a thiophene nucleus. This class of materials is inclusive of alkyl-substituted thiophenes, their corresponding sulfide, oxide, selenide, sulfonate, sulfonamide and nitro derivatives. For example, the alkyl-substituted thiophenes may be represented by the general formula:



wherein  $R^1$ ,  $R^2$ ,  $R^3$  and  $R^4$  are selected from the group consisting of hydrogen and substituted and unsubstituted alkyl, alkaryl, aryl, and aralkyl groups. The latter groups, as indicated, may carry one or more substituents such as sulfur, chlorine, hydroxy, nitro, sulfate, etc. It will be clear that at least one of the aforesaid  $R$  groups in the foregoing general formula will be an alkyl group such, for example, as butyl, amyl, octadecyl, paraffin wax, or the like. The sulfides, oxides, and selenide derivatives of the alkyl-substituted thiophenes will, of course, contain a sulfide, oxide or selenide bridge linking two or more thiophene nuclei. Typical of such materials is diethyl thiophene sulfide.

Illustrative of the preparation of typical thiophene compounds contemplated herein are those described in the following examples.

## 50 EXAMPLE I

## Paraffin wax-substituted dibutyl thiophene

A mixture consisting of 100 grams of dibutylthiophene, 260 grams of chlorinated paraffin wax containing 14 per cent by weight of chlorine (the paraffin wax has a molecular weight of about 350 and a melting point of about 126° F.) and 3 per cent by weight of anhydrous aluminum chloride, 55 was heated to a temperature of about 350° F. in

about one hour while stirring vigorously to avoid foaming induced by the evolution of hydrogen chloride. The mixture was maintained at this temperature for another hour while still stirring to insure complete reaction. Stirring was discontinued when hydrogen chloride was no longer evolved from the mixture. To purify the reaction mixture the latter was cooled to a temperature of 150-200° F., and an amount of water equal to about one-quarter the volume of the reaction mixture was added. About 3 per cent by weight of zinc dust was then added and the resulting reaction mixture was stirred for about 30 minutes. During this latter treatment, the reaction mixture was decolorized and the aluminum chloride therein was dissolved in the water layer which separated, the water layer was then removed and the remaining reaction mixture was washed with several portions of water. Butanol was used in conjunction with the water to break emulsions which formed. The water-washed reaction mixture was heated to remove the butanol and any residual water. The product thus obtained was predominantly paraffin wax-substituted dibutylthiophene and was characterized by the following properties: A. P. I. gravity 24.6; viscosity index 116.9; sulfur content 4.9 per cent by weight; molecular weight 557; pour point (A. S. T. M.) +80° F.

#### EXAMPLE II

##### Paraffin wax-substituted thiophene

A paraffin wax having a melting point of about 126° F., a molecular weight of about 350, and containing at least 20 carbon atoms with an average of 24 carbon atoms, was chlorinated by bubbling chlorine therethrough until the weight of the wax had increased by about 13 per cent. Two hundred

about 400° F. to remove any unreacted thiophene. The reaction product is predominantly mono-paraffin wax thiophene and is characterized by the following: A. P. I. gravity 25.8; viscosity index 137.0; 6.26 per cent sulfur; molecular weight of 456 and a pour point of 80° F.

It will be noted that the pour points of the products obtained in Examples I and II above are relatively high. These materials contain some free paraffin wax and can be dewaxed by the usual methods for dewaxing mineral oil lubricants. The dewaxed materials, those from which substantially all free paraffin wax has been removed, have sufficiently low pour points to be used as synthetic oils. For example, the mono-paraffin wax thiophene prepared in Example II above was dewaxed by diluting the same with 600 per cent by weight of methyl ethyl ketone followed by cooling the resulting mixture to 0° F. and filtering the cooled mixture at 0° F. The filtrate thus obtained was distilled to remove the methyl ethyl ketone and to obtain a product substantially free of paraffin wax. The mono-paraffin wax thiophene thus obtained had a pour point of +20° F.

The synergistic effect of the aforesaid phosphorus-containing and thiophene type characterizing agents is demonstrated by the Lauson engine test data presented in Table 1 below. The Lauson engine test is an operation test and involves operating a single cylinder Lauson engine for 36 hours at an oil temperature of 290° F. and a jacket temperature of 212° F. The oil used is a solvent-refined oil having a kinematic viscosity of 5.8 centistokes (S. U. V. of 45 seconds at 210° F.). After 36 hours of test, the acidity as represented by the neutralization number (N. N.) of the oil blend is measured.

Table 1

| Test No. | Characterizing Agent Added | Conc., Wt. Percent | N. N. | Per Cent Improvement | P/S Ratio |
|----------|----------------------------|--------------------|-------|----------------------|-----------|
| 1        | None                       |                    | 14.6  |                      |           |
| 1        | Dibutyl thiophene          | 0.4                | 13.5  | 7.5                  |           |
| 2        | None                       |                    | 8.4   |                      |           |
| 2        | Amylphenyl-phosphite       | 0.43               | 5.1   | 39                   |           |
| 3        | None                       |                    | 11.4  |                      |           |
| 3        | Dibutylthiophene           | 0.4                | 0.6   | 95                   | 0.4       |
| 4        | Amylphenyl phosphite       | 0.43               |       |                      |           |
| 4        | None                       |                    | 10.0  |                      |           |
| 4        | Dibutyl thiophene          | 0.2                | 1.4   | 86.1                 | 0.8       |
| 5        | Amylphenyl phosphite       | 0.43               |       |                      |           |
| 5        | None                       |                    | 10.95 |                      |           |
| 5        | Dibutyl thiophene          | 0.8                | 0.8   | 92.7                 | 0.2       |
|          | Amylphenyl phosphite       | 0.43               |       |                      |           |

grams of the chlorinated paraffin wax so prepared was contacted with 45 grams of lime (CaO) and the resultant mixture was agitated and heated for about 5 hours at about 500° F. Hydrogen chloride was evolved during this treatment and was neutralized, to a large extent, by reaction with the lime thus forming CaCl<sub>2</sub>. The reaction mixture was filtered to remove the CaO-CaCl<sub>2</sub> mixture and to obtain the unsaturated paraffin wax or paraffin wax olefin. The iodine value of the paraffin wax olefin was about 100.

A mixture of 100 grams of the aforesaid paraffin wax olefin and 30 grams of thiophene was heated in an autoclave at about 400° F. for about 5 hours in the presence of about 10 per cent by weight of a synthetic clay catalyst. The catalyst comprises silica in association with alumina. The reaction mixture was cooled and filtered to remove the clay catalyst. The filtrate thus obtained was distilled to a maximum temperature of

It will be clear from the foregoing tabulation that the combination of dibutylthiophene and amylphenylphosphite is more than a mere additive combination, inasmuch as the degree of improvement is only of the order of 46 per cent as indicated by an oil blend containing the dibutylthiophene alone and an oil blend containing the amylphenylphosphite alone. The corresponding oil blend containing both materials in the same concentrations provides an improvement of 94.7 per cent. It is also evident from the foregoing test results that the relative concentrations of thiophene compound and phosphorus compound influences the degree of synergistic action. This relationship is expressed in terms of the phosphorus to sulfur ratio of the compounds used in the oil. With the foregoing combination of amylphenylphosphite and dibutylthiophene, it has been found that the opti-

mum phosphorus to sulfur ratio is of the order of 0.4 and it is preferred that this ratio be maintained between about 0.1 and 0.8.

Not only may the phosphorus-containing agent and the thiophene agent be incorporated singly in the oil, but they may also be reacted together prior to the incorporation in the oil. In either case, the effect is not an additive one but a synergistic effect.

The oil-soluble phosphorus-containing compounds are generally used in the oil in concentrations of the order of about 0.4 per cent to about 1 per cent and the thiophene type compounds may be used in amounts from about 0.2 per cent to about 1 per cent, with the relative concentrations being so proportioned that the preferred phosphorus to sulfur ratio discussed above is maintained. These characterizing agents may be used in viscous mineral oils, volatilized oils, synthetic oils, greases and fatty oils, such as corn oil, soybean oil, lard oil, and the like. It should be clear that these characterizing materials may also be blended, that is, used as blending agents, in oils of the aforesaid type in higher concentrations than those enumerated above. They may, for example, predominate in the blend. In addition, the phosphorus-containing materials and thiophene nuclear materials, contemplated herein, may also be used as synthetic lubricants free from oils such as recited above, in view of their unusual lubricating value.

It is to be understood that the present inven-

tion is not to be construed as limited to the foregoing illustrative examples but is to be construed broadly in the light of the language of the appended claims.

We claim:

1. A mineral oil composition comprising a major proportion of a viscous mineral oil fraction, a minor proportion, from about 0.4 per cent to about 1 per cent, of amyl phenyl phosphite and a minor proportion, from about 0.2 per cent to about 1 per cent, of dibutyl thiophene.

2. A mineral oil composition comprising a major proportion of a viscous mineral oil fraction, a minor proportion, from about 0.4 per cent to about 1 per cent, of an alkyl phenyl phosphite and a minor proportion, from about 0.2 per cent to about 1 per cent, of a lower alkyl-substituted thiophene.

ORLAND M. REIFF.  
HARRY J. ANDRESS, JR.

#### REFERENCES CITED

The following references are of record in the file of this patent:

| UNITED STATES PATENTS |                  |               |
|-----------------------|------------------|---------------|
| Number                | Name             | Date          |
| 2,160,293             | Shoemaker et al. | May 30, 1939  |
| 2,258,806             | Pier et al.      | Oct. 14, 1941 |
| 2,315,072             | Nelson et al.    | Mar. 30, 1943 |
| 2,413,353             | Hunter           | Dec. 31, 1946 |